

G. VIRNEBURG.

ABRASIVE.

APPLICATION FILED APR. 11, 1914.

1,141,371.

Patented June 1, 1915.



Witnesses:

Leonard E. Boque  
Cameron A. Whitsett

Inventor

George Virneburg  
By Brown, Hanson & Baetcher  
Attorneys

# UNITED STATES PATENT OFFICE.

GEORGE VIRNEBURG, OF CHICAGO, ILLINOIS.

## ABRASIVE

1,141,371.

Specification of Letters Patent. Patented June 1, 1915.

Application filed April 11, 1914. Serial No. 831,282.

*To all whom it may concern:*

Be it known that I, GEORGE VIRNEBURG, a subject of the Emperor of Germany, residing at Chicago, in the county of Cook and 5 State of Illinois, United States of America, have invented certain new and useful Improvements in Abrasives, of which the following is a full, clear, concise, and exact description, reference being had to the accompanying drawings, forming a part of this 10 specification.

My invention relates to abrasives and is particularly concerned with sand-paper, or sand-cloth, and other forms of abrasive 15 coated fabrics.

It is the object of my invention to produce an abrasive fabric which may be used effectively in a wet finishing, smoothing or rubbing process.

20 My invention assumes particular importance in the removal of paints, shellacs and varnishes from woodwork or other articles, where such removal is effected by the abrasive processes. In work of this kind, the 25 hardened shellac, varnish, or paint, or other coating, is frequently removed by the ordinary sand-papering process and, in fact, this is the method heretofore almost universally employed. However, the work is extremely 30 unhealthful, since the fine particles of shellac, varnish or paint, or similar material, which are dislodged in the process are naturally thrown into the air and are being constantly inhaled by the workmen. 35 The chemical properties of these materials are extremely injurious to the lungs and certain diseases have been prevalent among the finishers' trade, due to this cause.

It is well known that if this work is carried on "wet", the dislodged particles are 40 kept from being thrown into the air and the difficulty is removed, but another difficulty is immediately encountered, since the water which is employed disintegrates the sand-paper or sand-cloth so quickly that a great deal of paper or cloth is required for a particular piece of work and a great deal of time is lost in constantly employing new pieces of paper or cloth, and the annoyance 45 of this is so great that it is a question whether it is not as great an evil as the dry process.

However, my invention steps in and cures both evils by the provision of a sand-paper or sand-cloth, or other abrasive fabric, which 50 may be given prolonged use in the "wet",

process without disintegration. In other words, the abrasive fabric which my invention provides may be used as effectively wet or dry, so that the safeguard as to health 60 may be employed without incurring any substitute difficulties.

My invention thus resides in a process of treating ordinary sand-paper or sand-cloth, or other abrasive fabric, in a compound for 65 treating such paper or cloth, or other fabric, and finally in the manufactured article itself.

In the accompanying drawing, I illustrate an abrasive-coated fabric forming the 70 subject-matter of my invention.

Ordinary sand-paper or sand-cloth may be used, different degrees of fineness of the sand being, of course, available. This sand-paper or cloth comprises a rather stout back 75 of a proper fabric coated with hot glue and then sprinkled with sharp sand, and then left to cool and dry. The piece of abrasive-coated fabric is then dipped in, painted with, or has applied thereto in some other 80 suitable way, a compound which I have determined to be useful for my purpose by careful and prolonged experiment. While it is very possible that other compounds may be used and that other proportions than those hereinafter specifically set forth may be employed, I shall state specifically what my experiments brought me to in order that I may give those skilled in the art the best and most complete information. It will be 85 understood, of course, that the scope of my invention is to be measured by that of the appended claims and not by this specification, which I make in detail so far as possible so that those skilled in the art may be 90 duly advised.

The compound which I have specifically determined by experiment to be a successful one is a combination of three primary compounds, which I shall designate "A", "B", 100 and "C".

Compound "A" is as follows:

|           |        |     |
|-----------|--------|-----|
| Benzin    | 58.00% |     |
| Resin     | 41.50% | 105 |
| Lead oxid | .50%   |     |

Compound "B" is as follows:

|             |        |     |
|-------------|--------|-----|
| Benzin      | 48.00% |     |
| Resin       | 51.40% | 110 |
| Nickel oxid | .60%   |     |

Compound "C" is simply beeswax.

These three compounds are mixed together in the following proportions:

5      Compound "A" ----- 12.50%  
       Compound "B" ----- 75.00%  
       Compound "C" ----- 12.50%

- The mixture of these compounds is preferably conducted at a temperature of 80°-90° Fahr., and the treatment of the fabric, 10 which has first been coated with glue and the abrasive, is preferably conducted at the same temperature and, as before stated, this treatment may be by applying the compound to the abrasive-coated fabric by 15 means of a brush, or by dipping the fabric in the compound, or by some other suitable method. The fabric and the coating of glue is impregnated throughout by this waterproofing compound. After the application 20 of the compound to the abrasive-coated fabric, the fabric is left to dry and is then ready for use. By "fabric" I mean paper or cloth, etc., and I use this meaning in the appended claims.
- 25      The removal of varnish or paint is effectively carried out by using comfortably cool water and a sponge. The surface to be worked should be kept wet and the abrasive fabric used upon it at the same time with 30 considerable pressure. The fabric, due to its manufacture as above described, will not disintegrate, as I have found by test, and will be an effective abrasive for the accomplishment of the work. At the same time, 35 the work will be dustless and the workmen will be free to breathe pure air instead of air mixed with the harmful particles which a dry varnish or paint removing process necessarily forms.
- 40      I claim as new and desire to secure by Letters Patent:

1. An article of manufacture comprising a piece of fabric, a coating of glue, and a

coating of an abrasive, said fabric and coating being impregnated with a compound of 45 a metal and an oil.

2. As an article of manufacture, a piece of fabric, a coating of glue, and a coating of an abrasive, said fabric and coating being impregnated with a compound of an oil, 50 metal and wax.

3. An article of manufacture comprising a piece of fabric, a coating of glue, and a coating of an abrasive, said fabric and coating being impregnated with a compound of an oil, the oxid of a metal, resin, and wax. 55

4. As an article of manufacture, a piece of fabric, a coating of glue, and a coating of an abrasive, said fabric and coating being impregnated with a compound of benzin, 60 resin, lead oxid, nickel oxid, and beeswax.

5. An article of manufacture comprising a piece of fabric, a coating of glue, and a coating of an abrasive, said fabric and coating being impregnated with a compound of 65 a primary compound "A" consisting of benzin 58%, resin 41.5%, lead oxid .5%; a compound "B" consisting of benzin 48%, resin 51.4%, nickel oxid .6%; and beeswax.

6. An article of manufacture comprising 70 a piece of fabric, a coating of glue, and a coating of an abrasive, said fabric and coating being impregnated with a compound of a primary compound "A" consisting of benzin 58%, resin 41.5%, lead oxid .5%; a compound "B" consisting of benzin 48%, resin 51.4%, nickel oxid .6%; and beeswax; the main compound comprising 12.5% of compound "A," 75% of compound "B" and 12.5% beeswax. 75

In witness whereof, I hereunto subscribe my name this 9th day of April, A. D., 1914.

GEORGE VIRNEBURG.

Witnesses:

LESLIE W. FRICKE.

CAMERON A. WHITSETT.